

## UNITED STATES PATENT OFFICE

2,171,791

PROCESS FOR RENDERING TEXTILES  
WATER REPELLENT

Walther Kaase and Ernst Waltmann, Krefeld,  
Germany, assignors to Heberlein Patent Cor-  
poration, New York, N. Y., a corporation of  
New York

No Drawing. Application May 13, 1936, Serial  
No. 79,496. In Germany May 16, 1935

12 Claims. (Cl. 8—113)

This invention relates to increasing water-re-  
pellence in textile materials.

For rendering certain textiles water-repellent  
there have been suggested processes which are  
based mainly on the surface treatment of the  
said materials with fatty-acid chlorides and fatty-  
acid anhydrides. In the carrying out of these  
prior processes however difficulties have been en-  
countered and the appearance and feel of the  
goods have been changed. These processes also  
required considerable time for their operation,  
requiring several hours to produce the results ob-  
tained.

The principal object of the present invention is  
15 to provide a simple process to increase water-re-  
sistance in various textile materials including cot-  
ton, jute, linen, hemp and various artificial silks  
and wool in a considerably shorter length of time  
with correspondingly less expénsé than that of  
20 the chlorides and anhydrides mentioned; and to  
produce materials having improved characteristics  
thereby.

The invention accordingly comprises the novel  
processes and steps of processes, specific embodi-  
25 ments of which are described hereinafter by way  
of example and in accordance with which we now  
prefer to practice the invention.

In our copending application Ser. No. 66,498,  
filed February 29, 1936, we have described and  
30 claimed the use of asymmetric fatty-acid anhy-  
drides containing a long acyl radical of at least  
10 carbon atoms and a considerably shorter acyl  
radical. In that copending application we have  
35 pointed out the use of asymmetric fatty-acid an-  
hydrides as applicable to various textile materials  
and have mentioned specifically cellulose-contain-  
ing materials for treatment. We have now found  
that wool may also be subjected to the process  
40 described in said copending application, the ma-  
terials employed and the conditions of treatment  
being otherwise substantially the same as men-  
tioned in said application.

In the present application we describe and claim  
45 the use for producing water-repellence in textiles,  
particularly cellulose-containing and wool ma-  
terials of unsymmetrical fatty-acid anhydrides of  
the general formula



In the formula  $R_1$  represents a fatty-acid radical  
containing at least 10 carbon atoms in a straight  
55 or derived chain or a naphthenic acid radical con-

taining at least 10 carbon atoms regardless of  
substitutions in such chain or ring.  $R_2$  repre-  
5 sents a radical containing at least 1 carbon atom  
and that part of the anhydride represented by  
the formula  $R_2.O.C:O$  is volatile when heated in  
the presence of the textile material preferably at  
temperatures of over about 100° C. The number  
10 of carbon atoms in  $R_2$  may be increased so long  
as the material is not prevented from volatilizing  
in the presence of the textile at temperatures  
15 below the point where the textile material would  
be injured. We also claim herein broadly the  
treatment of wool with the materials described  
in said copending application Ser. No. 66,498.

Substances falling under the above formula with  
their structural formulae are as follows:

Unsymmetrical stearic-acid carbonic-acid ethyl-  
ester anhydride having the structural formula



Unsymmetrical palmitic-acid carbonic-acid butyl-  
ester anhydride having the structural formula



Unsymmetrical adipic-acid cetyl-alcohol-ester  
carbonic-acid ethyl-ester anhydride having the  
30 structural formula



Unsymmetrical stearic-acid carbonic-acid meth-  
yl-ester anhydride having the structural formula



Unsymmetrical behenic-acid-carbonic-acid meth-  
yl-ester anhydride having the structural formula



These compounds may be prepared according to  
known methods for conversion of fatty-acids of  
50 the kind mentioned above with chloro-carbonic-  
acid alkyl-esters, as described by E. Fischer  
(Berichte 46, 2659) and German Patent 117,267.

The straight carbon chain of  $R_1$  may be in-  
terrupted by atoms or atomic groups O, S, N, 55

CO.O, O.CO, NR, NR.CO, CO.NR, SO<sub>2</sub>, NR.SO<sub>2</sub>, SO<sub>2</sub>.NR, in which R may be equal to hydrogen or any desired hydrogen or any desired hydrocarbon radical such as shown in the following formulae:



10 Palmityl-methyl-amino - acetic - acid - carbonic - acid methyl-ester anhydride;



15 Heptadecylamino - acetic - acid - carbonic - acid methyl-ester anhydride;



25 Dodecylaminobenzoic-acid-carbonic-acid methyl-ester anhydride.

30 The impregnation of the textile material with the anhydrides described may be performed in any desired manner, with or without the employment of organic solvents by means of soaking, spraying or the like. The products claimed may also be converted into an aqueous solution by means of suitable emulsifiers and as prepared in aqueous solution, may be employed for impregnation of the textiles.

35 The materials generally and specifically mentioned above as employed in the carrying out of our invention may be used for the impregnation of various textile materials including cellulose-containing materials such as cotton, jute, linen, 40 hemp or rayon, including viscose, cuprammonium or other precipitated cellulose or derivatives of cellulose such as acetyl cellulose and also wool. The materials may be treated in the form of fibers, yarns, fabric or other manufactured products.

45 In the case of acetyl cellulose the materials herein mentioned may be added to the spinning solution itself, thus combining the process of rendering water-repellent with the spinning process.

50 In carrying out the invention, catalysts such as pyridine may be employed, although they are not absolutely necessary.

55 The following are examples of embodiments of the invention as we now prefer to practice it. The invention is not to be restricted thereto except as indicated in the appended claims.

*Examples*

60 1. A linen fabric dyed with indanthrene is passed through an 0.5% solution of unsymmetrical stearic-acid carbonic-acid ethyl-ester anhydride in benzine at room temperature and after evaporation of the benzine is subjected 65 to 60 minutes to a temperature of 110° C.

65 2. A viscose satin having a warp of viscose and a filler of viscose crepe is passed through a 1% solution of unsymmetrical palmitic-acid carbonic-acid butyl-ester anhydride in benzine 70 at room temperature, and after evaporation of benzine is immediately subjected for 5 minutes to a temperature of 140° C.

70 3. A printed matt crepe having a warp of spinning-matt acetate silk and a filler of viscose 75 crepe is passed through a 1% solution of unsym-

metrical adipic-acid cetyl alcohol-ester carbonic-acid ethyl-ester anhydride in benzine at room temperature, and after evaporation of benzine is immediately subjected for 2 minutes to a temperature of 140° C.

5 4. Wool muslin is sprayed with a 2% solution of stearic-acid carbonic-acid methyl-ester anhydride in benzine, the solvent evaporated and the fabric subjected for 60 minutes to a temperature of 90° C.

10 5. A wool muslin is passed through a 1% solution of asymmetric-stearic-acid-acetic acid anhydride in benzine at room temperature, said anhydride having the structural formula



20 which is a substance having 2 acyl radicals, one acyl radical of more than 10 carbon atoms and the other of not more than 4 carbon atoms; the muslin is then suction filtered and thereupon exposed for 5 minutes to a temperature of 100° C. This is followed by a treatment at 150° C. 25 for 5 minutes.

6 A wool muslin is sprayed with a 1% solution of adipic-acid-stearic-alcohol ester-acetic acid anhydride having the structural formula



35 in benzine, and thereupon treated for 4 minutes at 100° C. This is followed by treatment at 100° C. for 5 minutes.

7 A velvet from mercerized cotton is passed through a 1% solution of unsymmetrical octocosan-acid-carbonic-acid-ethyl-ester anhydride in benzine at room temperature, and after evaporation of benzine is immediately subjected 40 for 2 minutes to a temperature of 140° C.

8 A clothing material consisting of acetate silk as warp and viscose crepe as weft is sprayed with a 0.5% solution of behenic-acid-carbonic-acid methyl-ester anhydride in benzine, the solvent evaporated and the fabric subjected for 60 minutes to a temperature of 110° C.

9 A cotton tent-cloth is passed through a 1% solution of naphthenic-acid-carbonic-acid methyl-ester anhydride in benzine, the solvent evaporated and the fabric subjected for 60 minutes to a temperature of 100° C.

10 To 1000 liters of a 20% solution of acetyl cellulose in acetone 1000 grams of stearic-acid-carbonic-acid methyl-ester anhydride are added and this mixture spun as usual in order to produce water-repellence in the spun filaments.

15 The process of the invention particularly as set forth in the specific embodiments above can be carried out with simple apparatus at relatively small expense and in a relatively short time. The products show an improved appearance, their feel as compared with similar untreated material is not substantially altered, and have a high degree of water-repellence which does not rapidly disappear upon cleansing by laundering or dry-cleaning.

20 In the claims where the expression "cellulose-containing material" is employed it is intended to cover fibers, yarns, fabrics or other forms of cotton, jute, linen, hemp or rayon including viscose, cuprammonium, or other precipitated cellulose or derivatives of cellulose such as acetyl cellulose.

The expression "textile material" as used in the claims is intended to cover such cellulose-containing material, as well as wool.

The expression "fatty-acid radical" as employed in the claims is intended to cover not only a straight carbon chain but also naphthenic acid ring structures, each of which may be substituted or unsubstituted by aliphatic or aromatic groups.

10 While the invention has been described in detail according to the preferred manner of carrying out the process, it will be obvious to those skilled in the art after understanding the invention, that changes and modifications may be made therein without departing from the spirit or scope of the invention, and it is intended in the appended claims to cover all such changes and modifications.

What is claimed as new and desired to be secured by Letters Patent is:

20 1. A process for the ennobling of textile material which comprises heating the textile material with an unsymmetric fatty-acid carbonic-acid ester anhydride, the fatty acid radical having at least ten carbon atoms and the carbonic-acid ester having at least two carbon atoms to volatilize the carbonic-acid radical having the lower number of carbon atoms, and to increase the water-repellence of said textile material.

25 2. A process for the ennobling of textile material which comprises treating the textile material with an unsymmetric fatty-acid carbonic-acid ester anhydride, the fatty acid radical having at least 10 carbon atoms and the carbonic-acid ester radical having at least 2 carbon atoms, removable by heating without injury to said textile material, and heating the textile material to a temperature above about 100° C. for several minutes to remove said last named radical 40 to increase the water-repellence and to decrease tendency to spotting of said material.

30 3. A process according to claim 3 in which the anhydride is combined with the textile material in solution and is thereafter heated for several minutes at a temperature above about 100° C. to 45 cause partial esterification of the material to produce a water-repellent property in said material.

35 4. A process for the ennobling of cellulose-containing material which comprises heating the cellulose-containing material with an anhydride to a temperature of the order of 90°-160° C. for a sufficient time to cause a reaction therebetween, said anhydride being an unsymmetric fatty-acid carbonic-acid ester anhydride, the fatty-acid radical having at least 10 carbon atoms therein and the ester radical having at least two carbon atoms therein, said heating causing removal 50 of said last-named radical, to increase the water-repellent property of the cellulose-containing material.

55 5. A process according to claim 4 in which wool is substituted for said cellulose-containing material.

60 6. A process for ennobling cellulose-containing material which comprises passing linen through a solution of unsymmetrical stearic-acid carbonic-acid ethyl-ester anhydride, and thereafter subjecting the treated linen for several minutes to a temperature of about 100-130° C.

70 7. A process for ennobling cellulose-contain-

ing material which comprises treating an artificial silk material with a solution of unsymmetrical palmitic-acid carbonic-acid butyl-ester anhydride, and thereafter subjecting the treated material for several minutes to a temperature of about 100-130° C.

8. A process for ennobling textile material which comprises subjecting wool to a solution of stearic-acid carbonic-acid methyl-ester anhydride, and thereafter subjecting the treated wool to a temperature of about 100-130° C.

9. A process for the ennobling of textile material which comprises heating the textile material with an unsymmetric fatty-acid carbonic-acid alkyl-ester anhydride of the general formula



20 in which  $R_1$  represents a radical containing an aliphatic group of at least ten carbon atoms and  $R_2$  a radical having an aliphatic member of at least one carbon atom, said heating being conducted at a temperature to split off the radical containing the lower member of carbon atoms and to cause the remainder of the anhydride to react with the textile material to increase the water-repellence thereof.

25 10. A process for the ennobling of wool which comprises heating the wool with an asymmetric fatty-acid anhydride containing a long acyl radical of at least ten carbon atoms and a considerably shorter acyl radical, said heating being conducted at a temperature to cause the shorter acyl radical to volatilize and the remainder of the anhydride to react with the wool to increase the water-repellence and decrease tendency of spotting of said wool.

30 11. A process for the ennobling of wool which comprises treating wool with an asymmetric fatty-acid anhydride having an acyl radical of at least 10 carbon atoms and the other acyl radical having not more than 4 carbon atoms and heating the wool so treated to volatilize the acyl radical having the lower number of carbon atoms, to increase the water-repellence and to decrease tendency to spotting of said wool.

35 12. A process for the ennobling of textile materials which comprises heating the textile material with an unsymmetric fatty-acid carbonic-acid alkyl-ester anhydride of the general formula



40 in which formula  $R_1$  represents a radical of at least 10 carbon atoms interrupted by atoms or atomic groups O, S, N, CO.O, O.CO, NR, NR.CO, CO.NR, SO<sub>2</sub>, NR.SO<sub>2</sub>, SO<sub>2</sub>.NR, in which R may be equal to hydrogen or any desired hydrocarbon radical, and  $R_2$  a radical having at least 1 carbon atom, said heating being conducted to volatilize said radical having the smaller number of carbon atoms and to cause the remainder of the anhydride to react with the textile material to increase the water-repellence of said textile material.

45 WALThER KAASE.  
ERNST WALTmann.

20

25

30

35

40

45

50

55

60

65

70

CERTIFICATE OF CORRECTION.

Patent No. 2,171,791.

September 5, 1939.

WALTHER KAASE, ET AL.

It is hereby certified that error appears in the printed specification of the above numbered patent requiring correction as follows: Page 2, first column, line 3, strike out the words "hydrogen or any desired"; and second column, line 35, for "100°" second occurrence, read 160°; page 3, first column, line 42, claim 3, for the claim reference numeral "3" read 2; and second column, line 42, claim 11, for "on" read one; and that the said Letters Patent should be read with this correction therein that the same may conform to the record of the case in the Patent Office.

Signed and sealed this 3rd day of October, A. D. 1939.

(Seal)

Henry Van Arsdale,  
Acting Commissioner of Patents.